

1,271,560.

C. H. FULTON.

APPARATUS AND METHOD FOR CONDENSING ZINC VAPOR  
APPLICATION FILED JAN. 8, 1917.

Patented July 9, 1918.

3 SHEETS-SHEET 1.

*Fig. 1.*



Inventor,  
Charles H. Fulton.  
By Beckwell & French Atty's.

C. H. FULTON.

APPARATUS AND METHOD FOR CONDENSING ZINC VAPOR.

APPLICATION FILED JAN. 8, 1917.

1,271,560.

Patented July 9, 1918.

3 SHEETS—SHEET 2.

Fig. 2.



Fig. 3.



Inventor,  
Charles H. Fulton.  
By Bakewell, Church & Attys

C. H. FULTON.

APPARATUS AND METHOD FOR CONDENSING ZINC VAPOR.  
APPLICATION FILED JAN. 8, 1917.

1,271,560.

Patented July 9, 1918.

3 SHEETS--SHEET 3.

Fig. 4



Fig. 5.



Inventor,  
Charles H. Fulton.  
By Bapewell & Church, Atty's.

# UNITED STATES PATENT OFFICE.

CHARLES H. FULTON, OF ST. LOUIS, MISSOURI, ASSIGNOR, BY MESNE ASSIGNMENTS, TO METALLURGICAL LABORATORIES, INCORPORATED, OF CHICAGO, ILLINOIS, A CORPORATION OF ILLINOIS.

## APPARATUS AND METHOD FOR CONDENSING ZINC-VAPOR.

1,271,560.

Specification of Letters Patent.

Patented July 9, 1918.

Application filed January 8, 1917. Serial No. 141,177.

*To all whom it may concern:*

Be it known that I, CHARLES H. FULTON, a citizen of the United States, residing at St. Louis, Missouri, have invented a certain 5 new and useful Improvement in Apparatus and Methods for Condensing Zinc-Vapor, of which the following is a full, clear, and exact description, such as will enable others skilled in the art to which it appertains to 10 make and use the same.

This invention relates to the condensation of zinc vapor.

In the condensation of zinc vapor into liquid spelter the products of distillation 15 that enter the condenser from the retort or distilling apparatus usually consists of substantially equal volumes of zinc vapor and CO at a temperature of approximately 1000 to 1300° C. In a mixture of zinc vapor 20 and CO of the above composition, no condensation to liquid zinc takes place until the temperature has dropped to approximately 870° C. It then begins and continues until a temperature of 419° C., the melting point 25 of zinc, is reached. Theoretically, therefore, the temperature of the condenser should range between 870° C. and 419° C., but for practical purposes, the temperature at the spelter tap of the condenser should not be 30 less than 500° C., so as to insure the discharge of liquid spelter. It is also desirable that the cooling of the gases from the temperature at which they enter the condenser down to 500° C. should be gradual, 35 rather than rapid.

The heat liberated by the condensation of the zinc vapor serves to heat the condensing surfaces of the condenser. The condenser loses heat by radiation into the atmosphere, 40 and unless the condenser construction is such that the input of heat is balanced by the outgo, it is evident that in order to maintain the proper temperature within the condenser, it is necessary to either heat or cool 45 the condenser, dependent upon the relation of the amount of heat radiated to that liberated by the condensation of vapor. Another important consideration in the condensation of zinc vapor to liquid metal is the amount 50 of surface that is necessary for the condensa-

tion of a given quantity of zinc vapor. And still another important consideration is the velocity or rate of flow of the zinc vapor over the condensing surfaces of the condenser.

One object of my present invention is to provide a practicable zinc condenser that can be built in large sizes and which is so designed that the condensing surfaces can either be heated or cooled, thereby making 55 it possible to keep the condenser within the proper temperature range.

Another object is to provide a condenser which is so constructed that the zinc vapor will have a certain definite velocity of flow 60 over condensing surfaces upon which liquid zinc has been formed, the contact of vapor with liquid zinc materially aiding the condensation.

As previously stated, the temperature of 70 the condenser should range between 870° C. and 500° C., and while it is possible to maintain this temperature range with a condenser constructed in accordance with my invention, I have discovered that if zinc vapor 75 is passed through a condenser which is maintained at such a temperature that less than the usual percentage of zinc will be condensed to the liquid form and said vapor thereafter admitted to another condenser 80 whose condensing surfaces are maintained at a lower temperature and within a different temperature range that the condensing operation can be controlled more easily than is possible when the condensing operation is 85 carried on in a single condenser whose temperature ranges between 870° C. and 500° C. Therefore, another object of my present invention is to provide a method of condensing zinc vapor that can be easily controlled. 90

Briefly described, my improved condenser consists of a relatively long passageway through which the gas stream from the distilling apparatus travels, condensing surfaces in said passageway upon which so-called "nuclei" of zinc gather and over which the gas stream sweeps while traveling through the passageway at a definite velocity, and means for either heating or cooling said condensing surfaces. 100

My improved method, briefly stated, consists in causing the gas stream or products of distillation from a zinc distilling apparatus to pass through a condenser or condensing chamber that is maintained at a sufficiently high temperature to cause part of the zinc in said stream to be condensed to liquid spelter, and thereafter, causing said gas stream to enter a condenser or condensing chamber that is maintained at a lower temperature, so as to convert some of the zinc vapor into liquid spelter and the remainder into "blue powder." It is immaterial what particular type of condensers or condensing chambers are used in practising my method, and while I have herein illustrated an apparatus for practising my method which consists of a plurality of my improved condensers connected up in tandem relation, I wish it to be understood that my improved method is not limited to use with an apparatus of the particular construction herein shown.

Figure 1 of the drawings is a vertical sectional view illustrating a condenser constructed in accordance with my invention and connected in tandem relation with a condenser of somewhat similar design, so as to produce an apparatus for practising my novel method above described.

Figs. 2 and 3 are horizontal sectional views, taken on the lines 2-2 and 3-3 of Fig. 1.

Fig. 4 is a vertical sectional view, taken on the line 4-4 of Fig. 1; and

Fig. 5 is a development of the tubular members that form the outer shells of the condensers shown in Fig. 1, illustrating the arrangement of the baffles or vanes in the passageways of the condenser A through which the zinc vapor travels.

Referring to the drawings, which illustrate the preferred form of my invention, A and B designate two zinc condensers that are arranged in tandem relation, or in such a manner that a gas stream or products of distillation from a zinc distilling apparatus will travel through the condenser A, and thereafter, enter the condenser B. The condenser B is similar in general design to the condenser A, but it is smaller and the annular portion of the condensing passageway of same is not provided with baffles. Each condenser comprises a base 1 that is preferably built up of refractory material, a tubular-shaped member 2 of any preferred cross-sectional form arranged on the base 1 in an upright position, so as to form the outer wall or shell of the condenser, a tubular-shaped member 3 arranged inside of the member 2 and spaced away from the side walls of same, so as to form a passageway Y through which the gas stream travels, and a tubular-shaped member 4 arranged inside

of the member 3 and spaced away therefrom, so as to form a flue X through which a cooling or heating medium can circulate. The members 2, 3 and 4 are preferably formed from refractory material and are of cylindrical shape in cross section, and the inner member 4 is so arranged that it forms part of the passageway through which the gas stream flows. The upper ends of the members 2 and 4 are closed and the interior of the member 4 is connected with the passageway Y formed between the members 2 and 3 by means of a duct 5, as shown in Fig. 1, that leads from the upper end of the member 4 into said passageway. The lower end of the member 4 communicates with a duct 6 in the base 1 of the condenser, to which the gas stream from the distilling apparatus is supplied, as hereinafter described, so that said gas stream will circulate upwardly through the member 4 to the duct 5 that leads from the upper end of said member, and thence through said duct to the annular passageway Y between the members 2 and 3. Baffles 7 that are arranged in the passageway Y of the condenser A serve as condensing surfaces over which the gas stream sweeps when the condenser is in operation, and members 8 are arranged inside of the member 4, so as to retard the passage of the gas stream through said member 4 and also serve as condensing surfaces, the baffle members 8 preferably consisting of flat plates of refractory material that are arranged horizontally, one above the other in staggered relation, as shown in Figs. 1 and 2, and supported by struts or uprights 9 which may consist of short sections of pipe made of refractory material. The baffles 7 in the annular portion Y of the condensing passageway preferably consist of inclined vanes that extend spirally around the member 3 at an angle of approximately 90°, said vanes being so arranged that the gas stream will follow a tortuous path after entering the passageway Y. As shown in Fig. 5, two of the vanes 7 that extend downwardly from the upper end of the passageway Y terminate a short distance from the bottom of said passageway, and the two intermediate vanes 7 extend upwardly from the bottom of said passageway and terminate a short distance from the upper end of same, thus causing the gas stream to follow the path indicated by the arrows in Fig. 5. In the condenser A herein shown a fifth baffle or vane 7a extends throughout the entire height of the passageway Y from the lower to the upper end of same, so as to form a dividing wall between the inlet port, where the gas stream enters the passageway X, and the outlet port, where said gas stream leaves said passageway. At the lower end of the passageway Y are one

or more ports 10 through which the spelter can be drawn out of said passageway, and when the condenser A is arranged in tandem relation with another condenser B, so as to 5 produce an apparatus for practising the method that forms one feature of my present invention, a gas outlet duct 11 is provided for conducting the gas stream from the lower end of the passageway Y of the 10 condenser A into the duct 6 in the base of the condenser B, the gas stream passing from said duct 6 upwardly through the member 4 of the condenser B, and thence through the duct 5 to the upper end of the 15 passageway Y of the condenser B, as shown diagrammatically in Fig. 5. If the condenser A is used alone, or not in combination with another condenser, as shown in Fig. 1, ports (not shown) will be provided at the 20 upper end of the passageway Y of the condenser A through which the carbon monoxid gas can escape, but when said condenser A is arranged in tandem relation with another condenser B, as herein shown, the passageway Y of the condenser A will not be provided with discharge ports for the carbon monoxid gas, but, on the contrary, carbon monoxid gas discharge ports will be provided only in the condenser B, preferably 25 at the upper end of the passageway Y of said condenser B, as indicated by the reference character 12 in Fig. 5.

The condensing surfaces of the condenser A can be maintained at the proper temperature by supplying either a heating medium or a cooling medium to the annular flue X between the two tubular-shaped members 3 and 4, the upper end of said flue communicating with the atmosphere through an 30 opening 13 formed in a removable cover 14 at the upper end of said flue, as shown in Fig. 1. The lower end of the flue X communicates with a chamber Z formed in the base of the condenser, and a duct 15 leads 35 from said chamber Z, as shown in Fig. 3, to a chamber W formed in the base of the condenser that serves either as a combustion chamber or as an air chamber, dependent upon whether the condenser is being heated 40 or cooled. If desired, a checkerwork of brick 16 can be arranged in the annular flue X, as shown in Figs. 1 and 2, so as to absorb heat from the products of combustion, or the heated air that is supplied to said flue under 45 certain conditions, and thus assist in maintaining the condensing surfaces in the member 4 and in the passageway Y at the proper temperature. The chamber W in the base of the condenser is preferably arranged below 50 a passageway 17 in said base through which the gas stream travels in passing to the duct 6, and said passageway 17 is connected by means of a port 18 with a supply duct 19 that leads from a retort or distilling appa-

ratus (not shown). If desired, a valve 20 65 can be provided for controlling the port 19. The duct 6 that leads from the passageway 17 to the lower end of the tubular-shaped member 4 slopes downwardly toward the passageway 17, as shown in Fig. 1, so as 70 to conduct spelter from the member 4 to said passageway, and a spelter tap 17<sup>a</sup> is formed in one end of the passageway 17, as shown in Fig. 4, so as to permit the liquid metal to be drawn from same. 75

The chamber W is provided in its end walls with openings 21 that are adapted to serve either as burner ports or air supply holes, and baffles 22 are arranged in said chamber W in zig-zag relation or in any 80 other preferred manner, so as to direct the heating medium or the cooling medium into the passageway 15 that leads to the chamber Z in the base of the condenser with which the lower end of the flue X communicates. 85 Generally speaking, under normal operations, cooling of the condenser will be necessary, and at such times, air is supplied to the chamber W by fans or other suitable devices that are connected up with the openings 21 in the end walls of the chamber W. 90

Assuming that the gas stream or the products of the distillation of the ore charge, consisting of approximately equal volumes of zinc vapor and carbon monoxid gas, enter 95 the condenser A at a temperature of approximately 1050° C., and that the carbon monoxid gas leaves the condenser at a temperature of approximately 600° C., there is liberated, by each pound of zinc condensed, 1051 B. T. U. For purposes of calculation assuming an ore charge that contains 774 lbs. of zinc, this amounts to 813,474 B. T. U., or 135,575 B. T. U. per hour for a six hour distillation period. This is equivalent to 33,894,000 small calories per hour. Assuming that the interior condensing surfaces are at the proper temperature, there must therefore be dissipated every hour this quantity of heat. The dissipation of this 100 heat will take place by radiation from the exterior surface of the condenser and the interior flue surface of the condenser. Whether the condenser must be heated or cooled will depend upon the amount of heat 105 which is radiated from it. If the amount of heat radiated from the condenser is greater than 34,000,000 calories per hour, the condenser will have to be heated, if not, it will have to be cooled. Assuming an interior 110 temperature in the center member 4 of 850° C., an exterior temperature in the central annular flue X of 200° C., an interior temperature in the annular passageway Y of 600° C. and an exterior temperature of the 115 outer wall 2 of the condenser of 200° C., the total amount of heat radiated per hour from the condenser, as constructed in cer-

tain size and of certain insulating and refractory material, will be 10,110,000 calories per hour. It is, therefore, apparent that there is an excess of heat amounting to 5 23,784,000 small calories per hour, which must be dissipated by increased cooling. In the condenser herein shown the cooling is effected by spraying water on the exterior wall of the condenser and by passing cool 10 air through the central annular flue X of the condenser.

This amount of cooling is necessary when the maximum supply of zinc vapor is being delivered to the condenser. When this 15 amount decreases, the amount of cooling will also decrease and a point may be reached, where, instead of cooling the condenser, it will be necessary to heat it. This heating is also necessary when the zinc distilling apparatus is started from the cold, in order to bring the condenser to the proper temperature. When heating is necessary, oil burners or other suitable devices are used in connection with the chamber W in the base of the 20 condenser to cause a heating medium to circulate upwardly through the flue X. Under normal conditions, however, it will be necessary to supply a cooling medium instead of a heating medium to the condenser, so as to 25 maintain the condensing surface at the proper temperature. As previously stated, the walls of the condenser are built of relatively poor heat-conducting material, such, for example, as fire brick, and if desired, 30 some portions of the condenser from which heat radiates may be covered with heat-insulating material, such, for example, as sil-o-cel, so that it will be possible to maintain a high temperature on one side of said portions and a relatively low temperature on 35 the other side and still have the proper amount of heat transfer. In actual practice the outer wall or shell of the condenser is preferably so proportioned and constructed 40 that the radiation loss will be balanced by the heat input, the outer wall or shell of the condenser A herein illustrated being composed of fire brick f protected on the outer side by a covering of sil-o-cel s.

50 As previously stated, one important consideration in the condensation of zinc vapor to liquid metal is the amount of surface that is necessary for the condensation of a given quantity of zinc vapor. In the condensation 55 of zinc vapor to liquid metal, as well as in the condensation of steam into water—so-called "nuclei of condensation" are necessary; that is, if there be provided in a space a large number of points or "nuclei" upon 60 which the vapor has been condensed into liquid, these small particles of liquid already formed facilitate the further condensation of the vapor. Some surface must be provided for these so-called "nuclei" to gather

on, and if a construction is obtained consisting of surfaces against which the zinc vapor is constantly swept, condensation is greatly facilitated. In my improved condenser the desirable results just referred to are accomplished by providing the condenser with a 65 relatively long condenser passageway that is equipped with condensing surfaces which are so designed that the zinc vapor follows a tortuous path, in traveling through said passageway and is constantly swept over 70 said surfaces, and furthermore, by providing the condenser with a flue through which a heating medium or cooling medium can be passed, so as to maintain said condensing surfaces at the proper temperature necessary to condense zinc vapor to liquid metal. 80

The temperature conditions under which zinc vapor will condense to liquid spelter are as follows:

| Relative<br>Zn. | Volumes<br>CO. | Partial pres-<br>sure of the<br>zinc.<br>Millimeters. | Temperature.<br>Degrees. | Per cent. of<br>total zinc<br>condensed. |
|-----------------|----------------|-------------------------------------------------------|--------------------------|------------------------------------------|
| 50              | 50             | 330                                                   | 362                      | None.                                    |
| 25              | 75             | 190                                                   | 390                      | 72%                                      |
| 20              | 80             | 152                                                   | 733                      | 72%                                      |
| 10              | 90             | 76                                                    | 726                      | 90%                                      |
| 5               | 95             | 35                                                    | 670                      | 96%                                      |

85 This means essentially, for example, that provided sufficient time is given, and surface 95 is offered, when the temperature is 800° C., 72% of the zinc will be condensed to the liquid form; or, when the temperature is about 725° C., 90% of the zinc will be condensed to liquid form. Now, the drop from 100 870° C. to 725° C. is only 145° C., and therefore, it is obvious that it is much easier to maintain a condenser within this range than to attempt to maintain it within the greater range necessary for complete condensation. Accordingly, I have devised a 105 method for condensing zinc vapor which is distinguished from the methods heretofore used, in that the condensation is effected by stages, or, in other words, 110 in a plurality of condensers having different temperature ranges, instead of in a single condenser having a temperature range from 870° C. to 500° C. In carrying 115 out said method I prefer to condense part of the zinc vapor in a condenser that is maintained at a rather high temperature, the range being preferably from 870° C. to 700° C., so that about 90% of the metal will be condensed as liquid spelter and completing the condensing operation in a second condenser that is operated relatively cool and which will produce some liquid spelter but mostly "blue powder." 120 The second condenser is preferably smaller than the first condenser and is arranged in tandem relation with same, and while any suitable type of condensers may be used in

practising my method, I prefer to use an apparatus of the kind herein illustrated, which is composed of two condensers A and B whose condensing chambers are connected together in such a manner that the gas stream, after traveling through the condenser A, will enter the condenser B. As shown in Fig. 1 of the drawings, the condenser A is provided with a gas stream 10 discharge passageway 11 that leads from the annular passageway Y of the condenser A into the heated passageway 17 in the base of the condenser B. The condenser B is of the same general design as the condenser A, 15 but the annular passageway Y of the condenser B is not provided with baffles or vanes. The condenser B is maintained at a temperature of approximately 700° C. at the inlet and 500° C. or less at the outlet, 20 so that some of the zinc vapor that enters same will be condensed as liquid metal in the inner tubular member 4 and the balance of said vapor will be converted into "blue powder" in the annular passageway Y, 25 said annular passageway being provided at its lower end with one or more clean-out openings that are normally closed by removable covers 24.

Having thus described my invention, 30 what I claim, and desire to secure by Letters Patent, is:

1. A zinc condenser provided with tubular-shaped members arranged one within the other and spaced apart so as to form a 35 passageway through which a gas stream from a zinc distilling apparatus travels.

2. A zinc condenser provided with a passageway through which a gas stream from a zinc distilling apparatus travels, 40 condensing surfaces in said passageway of such form and arrangement that the gas stream will travel through said passageway at a definite velocity and impinge upon or sweep over said condensing surfaces, and means whereby said passageway 45 may be either heated or cooled so as to control the temperature of said condensing surfaces.

3. A zinc condenser, comprising a flue 50 through which a medium can be passed to control the temperature of the condenser, a passageway surrounding said flue through which a gas stream from a zinc distilling apparatus travels, and condensing surfaces in said passageway that cause said stream of gas to follow a tortuous path in traveling through said passageway.

4. A zinc condenser, comprising a vertically-disposed structure provided with a 60 condensing passageway of substantially tubular form that extends longitudinally of same between the center and the periphery of said structure, and condensing surfaces in said passageway arranged in such a man-

ner that products of distillation that enter 65 said passageway will flow in a zig-zag path in traveling through said passageway.

5. A zinc condenser provided with a substantially annular-shaped passageway through which a stream of gas supplied to 70 the condenser flows, and baffles in said passageway that constitute condensing surfaces and which are so arranged that the gas will flow longitudinally of said passageway in opposite directions while traveling 75 circumferentially through same.

6. A zinc condenser provided with a substantially tubular-shaped passageway through which a gas stream from a zinc distilling apparatus flows, and means in 80 said passageway for causing the gas to flow longitudinally of said passageway in opposite directions and also follow a substantially spiral course in traveling through said passageway.

7. A zinc condenser provided with a substantially annular-shaped passageway that is adapted to receive a stream of gas from a zinc distilling apparatus, and substantially spirally-disposed vanes or baffles 90 in said passageway arranged in such a manner that the gas will follow a zig-zag course in traveling circumferentially through said passageway.

8. A zinc condenser provided with a 95 passageway through which a stream of gas from a zinc distilling apparatus flows, said passageway comprising one portion that is provided with baffles which tend to impede the flow of gas through same, and a different portion provided with substantially spirally-disposed baffles which cause the gas to be projected with considerable force against condensing surfaces.

9. A zinc condenser provided with a passageway through which a stream of gas containing zinc vapor flows, said passageway comprising communicating, centrally-arranged portions that are provided with members that serve as condensing surfaces 110 and also as baffles which cause the gas to sweep over said condensing surfaces.

10. A zinc condenser, comprising a vertically-disposed structure provided with an annular passageway that extends longitudinally of same, condensing surfaces in said passageway on which zinc "nuclei" form, and means for enabling heat to be absorbed from said condensing surfaces or additional heat put into same so as to accurately control the temperature of the condenser.

11. A zinc condenser provided with an annular condensing chamber whose outer wall is exposed to the atmosphere, and means for enabling the inner wall of said chamber 125 to be heated or cooled.

12. A zinc condenser provided with a condensing passageway that comprises a tubular

- portion arranged inside of an annular portion, and a flue between the two portions of said passageway through which a heating medium or cooling medium can be passed.
13. A zinc condenser provided with an annular flue to which a heating medium or a cooling medium can be supplied, and condensing surfaces on the interior and exterior of the flue which dissipate the heat produced by the condensation of the zinc vapor.
14. A zinc condenser formed by a plurality of tubular-shaped members arranged one within the other and spaced apart so as to form a flue that is interposed between communicating passageways through which a gas stream from a zinc distilling apparatus flows, said flue being adapted to be supplied with a heating medium or a cooling medium for the purpose specified.
15. A zinc condenser composed of a substantially tubular-shaped member closed at its opposite ends, an annular flue arranged inside of said member and spaced away from the side walls thereof so as to form an annular condensing passageway, a connection between said annular passageway and the space surrounded by said flue, means for supplying a stream of gas from a zinc distilling apparatus to the space surrounded by said flue, and means for supplying either a heating medium or a cooling medium to said flue.
16. A zinc condenser provided with a vertically-disposed, tubular-shaped member to which a stream of gas from a zinc distilling apparatus is supplied, an annular flue that surrounds said member, a shell that surrounds said flue, baffles arranged on the interior of said shell and on the interior of said tubular-shaped member, and means whereby either a heating medium or a cooling medium can be supplied to said flue.
17. A zinc condenser provided with a vertically-disposed, tubular-shaped member to which a stream of gas from a zinc distilling apparatus is supplied, an annular flue that surrounds said member, a shell that surrounds said flue, baffles arranged on the interior of said shell and on the interior of said tubular-shaped member, and means whereby either a heating medium or a cooling medium can be supplied to said flue, the baffles on the interior of said shell consist-
- ing of substantially spirally-disposed vanes, and the baffles on the interior of said tubular-shaped member being formed by substantially horizontally-disposed plates arranged one above the other and spaced apart.
18. A zinc condenser, comprising a base, a structure on said base provided with a passageway through which a stream of gas from a zinc distilling apparatus flows, a flue combined with said passageway, a chamber in said base that can be either heated or cooled, and a connection between said chamber and said flue.
19. A zinc condenser provided with a base that is equipped with a passageway through which a stream of gas being supplied to the condenser travels, and means for enabling said passageway to be either heated or cooled.
20. A zinc condenser, comprising a vertically-disposed structure provided with a passageway which is so formed that the products of distillation supplied to the condenser can flow longitudinally of said structure in opposite directions and also circumferentially through the structure, and means for enabling the temperature of said structure to be controlled.
21. A zinc condenser, comprising a base provided with means for enabling it to be either heated or cooled, a tubular-shaped member arranged on said base in an upright position and closed at its upper end so as to form the outer wall of the condenser, an annular flue arranged inside of said member and provided at its lower end with an inlet opening up through which a heating medium or a cooling medium from the base can circulate, and condensing surfaces arranged on opposite sides of said flue.
22. A zinc condenser, comprising a base, a chamber in said base that is adapted to serve as a combustion chamber or as a cool air supply chamber, a structure on said base provided with a gas passageway that comprises a central tubular-shaped portion that communicates with an annular portion which surrounds same, baffles in said passageway that serve as condensing surfaces, an annular flue arranged between the two portions of said passageway, and a connection between said flue and the chamber in said base.

CHARLES H. FULTON.